

# UNITED STATES PATENT OFFICE.

ALBERT CARLOS GRESSLE, OF HAMILTON, OHIO.

## COMPOUND FOR FORMING RUNNERS.

1,408,587.

Specification of Letters Patent. Patented Mar. 7, 1922.

No Drawing.

Application filed April 30, 1921. Serial No. 465,778.

To all whom it may concern:

Be it known that I, ALBERT CARLOS GRESSLE, a citizen of the United States, residing at Hamilton, in the county of Butler 5 and State of Ohio, have invented certain new and useful Improvements in Compounds for Forming Runners, of which the following is a specification.

This invention relates to compounds, and 10 particularly to a compound providing a substitute for fire clay, putty or woven asbestos and other "runners" used for dams for the pouring of lead joints on horizontal hub and spigot, water, gas and soil pipes, and 15 in pouring Babbitt metal bearings.

In the pouring of Babbitt metal bearings and in the pouring of lead joints in pipes, wet fire clay is commonly used, as is also putty and asbestos, but rolls made from 20 these materials and used as "runners" are unsatisfactory, in that the joint so made is rough and unsightly and there is great liability of leakage and these runners are difficult to apply.

25 One difficulty of these runners is to secure proper consistency under all service conditions. The object of this compound is to provide a material from which these rolls constituting runners may be made up which 30 always remains the same consistency, which will not blow or sputter, causing waste of material and loss of time, which is not affected by climatic changes, which will not soften materially and unduly with excessive 35 heat, which will last indefinitely and can be used over and over again. This compound preferably consists of the following ingredients in the following proportions:—

|                                                 |          |
|-------------------------------------------------|----------|
| Dry asbestos compound                           | 17.6 oz. |
| Strained linseed oil                            | 7 oz.    |
| Coal tar pitch or pitch of equivalent character | 2 oz.    |

40 This compound is mixed in a power driven mixer having agitating blades in a revolving tank. The various ingredients of the compound are thoroughly mixed to form a tough mass and is then kneaded to the proper consistency. The dry asbestos 45 compound is an asbestos compound commonly found on the market and consists of approximately 53.86% of asbestos, .81% of silica, .54% of oxide of iron and alumina, 20.20% of lime, .62% of magnesia, 13.94% 50 of carbon dioxide, 4.80% of sulphur trioxide, and 6.28% of water. The coal tar

pitch is a by-product of coal secured in the manufacture of coke and gas. I do not wish to be limited to the use of coal tar pitch, however, as other mineral pitch as asphaltum may be used in the compound. The linseed oil is of ordinary commercial character. I do not wish to be limited to the particular asbestos compound referred to, though this is particularly good for the purpose described, as other compounds of asbestos may be used. As before remarked, I do not wish to be limited to any particular kind of pitch, whether a coal tar product or a natural asphaltum or mineral pitch, 60 nor do I wish to be limited to the use of linseed oil, as other oils of an equivalent nature might be used for this purpose, though linseed oil has proved itself to be the best for the circumstances. Obviously 65 I do not wish to be limited to the exact proportions of the ingredients, as these proportions might be changed without departing from the spirit of the invention. Thus I may use from 14 to 18 ounces of dry asbestos, from 6 to 8 ounces of linseed oil, and from 1 to 4 ounces of coal tar pitch or pitch of equivalent character.

In use, the plastic mass produced by the formula above stated is worked in the hands 70 until it secures a proper consistency. It is then rolled to the desired length and thickness on a clean surface, and then is applied to the joint or bearing, the pour hole being built high enough to insure a perfect pour 75 and the edge of the roll being pressed well against the edge of the metal. The joint is then poured and after it is poured and set, the roll may be cleaned from the metal and then the material is pressed firmly together 80 and put back in the sealed container from which it was taken. If the compound should become too stiff for use, lubricating oil is added sufficient to bring it back to its original condition, the lubricating oil 85 being thoroughly mixed into the mass by kneading or working in any suitable manner.

Asbestos is used to form the body of the "runner" because it adds materially to the 90 tough or elastic properties of the body or compound and further because asbestos is refractory and, therefore, is not affected by the intense heat exposure. Furthermore, the fibrous nature of the asbestos when combined with a mixing medium renders the 95 mass very tenacious. Any finely ground

asbestos may be used but the composition asbestos before referred to is particularly satisfactory.

5 I do not wish to be limited to the use of linseed oil, as any other vegetable oil having practically the same characteristics as linseed oil may be used. Linseed oil is used in the compound because of its tendency to "gum" when exposed to air and this feature 10 in the linseed oil adds to the life of the compound because of the thin film of gum coating enveloping the same which protects the compound and tends to prevent it from hardening with exposure.

15 I have heretofore referred to the fact that lubricating oil may be mixed with the mass should it become too stiff. The term "lubricating oil" refers to the mineral oils which have a relatively high flashing point. This 20 mineral oil is used to soften the roll and is particularly desirable because it does not dry out readily, and moreover is easily obtained in almost any place. The coal tar pitch or asphaltum adds to the toughness of the compound. The reason why the compound remains in the same consistency is particularly 25 because of the use of linseed oil which gums upon exposure, as before stated.

30 A runner constructed in accordance with my invention will not blow or sputter because there is an absence of moisture. This is the difficulty with using wet clay rolls. Wet clay is particularly dangerous because 35 of the extreme moisture content, and moreover is not readily obtained. Climatic changes do not alter my compound because of its combination of oils and pitch which in combination resist the congealing effects 40 of relatively low temperatures. Excessive heat, on the other hand, will not soften the compound beyond use because of the refractory properties of the asbestos. The compound will last indefinitely because there is no wear on the compound and the only loss 45 is due to the carelessness of the operator.

50 My compound when made into a "runner" is better than a woven runner because of a certain amount of elasticity which it has and the ease with which it may be applied. Putty as a runner will break, burn through and blow out because of its weak texture and

sputter because of moisture, due to keeping the putty in water to prevent it from hardening. A runner constructed in accordance with my compound will eliminate rough and 55 unsightly joints such as are made where woven or rope runners are used. The hub ends of all cast iron pipe are rough and this makes it impossible to apply a woven runner without great leakage and rough pouring. 60 Furthermore, with my improved runner compound it is possible to build a high pour hole or gate which enables the operator to obtain a perfectly filled joint, whereas a woven runner necessitates so large and so 65 flat a pour hole or gate that molten metal rarely, if ever, finds its way to the extreme depth of joint, leaving a void which results in a leaky joint, or if babbitting leaves an imperfect bearing, making trouble and waste 70 of time. My compound being entirely plastic may be pressed firmly against irregular metal parts, preventing all leakage of metal while pouring.

I do not wish to be limited to the use of 75 the mineral pitch, as it is possible to form a compound for these runners consisting of a combination of dry finely ground asbestos and linseed oil, though this will not have the toughness, elasticity and other desirable 80 characteristics as will a compound composed of the asbestos, linseed oil and pitch.

I claim:—

1. A dam forming compound of the character described including dry asbestos 14 to 85 18 ounces, a vegetable oil 6 to 8 ounces, and from 1 to 4 ounces of mineral pitch.

2. A dam forming compound of the character described including finely ground dry asbestos 14 to 18 ounces, an oil which will 90 gum 6 to 8 ounces, and 1 to 4 ounces of mineral pitch.

3. A dam forming compound consisting of dry asbestos 17.6 ounces, oil 7 ounces, and mineral pitch 2 ounces.

4. A dam forming compound consisting of dry asbestos 17.6 ounces, linseed oil 7 ounces, and coal tar pitch 2 ounces.

In testimony whereof I hereunto affix my signature.

ALBERT CARLOS GRESSLE.